

W. P. THOMPSON.

PROCESS OF MANUFACTURING CERTAIN LEAD PRODUCTS.

APPLICATION FILED FEB. 6, 1915. RENEWED FEB. 5, 1919.

1,297,934.

Patented Mar. 18, 1919.



WILLIAM PHILLIPS THOMPSON.  
By

Stewart Mason

Attorneys.

Witnesses.

H. A. Dodge  
McGalliard

# UNITED STATES PATENT OFFICE.

WILLIAM P. THOMPSON, OF LIVERPOOL, ENGLAND.

## PROCESS OF MANUFACTURING CERTAIN LEAD PRODUCTS.

1,297,934.

Specification of Letters Patent. Patented Mar. 18, 1919.

Application filed February 6, 1915, Serial No. 6,607. Renewed February 5, 1919. Serial No. 275,199.

To all whom it may concern:

Be it known that I, WILLIAM PHILLIPS THOMPSON, a subject of the King of Great Britain, residing at Liverpool, in the county 5 of Lancaster, in the Kingdom of England, have invented certain new and useful Improvements in Processes of Manufacturing Certain Lead Products, of which the following is a specification.

10 This invention has for its principal object a very simple method of making white lead (hydro-carbonate of lead) from lead without touching the material from the time it is metallic lead, to the time when it is completely formed hydro-carbonate of lead, and at the same time producing a hydro-carbonate of lead almost if not quite equal to that produced by the Dutch process, but in a vastly shorter time, and also if desired an 15 intermediate product, pure or slightly hydrated finely divided non-crystalline mon-oxid of lead.

The invention is best described by aid of the accompanying drawings, in which:

20 Figure 1 shows a somewhat diagrammatic longitudinal vertical section of my preferred form of apparatus.

25 Fig. 2 is a cross sectional view of same, looking from the right of Fig. 1 with the chimney, oxidizing devices, the conveyer, the acetic acid chamber, the fan and air-heating pipes omitted.

30 Fig. 3 is an enlarged vertical section of the aspirating device and chamber on the same plane as Fig. 1,

35 Fig. 4 a plan view of the scraping device.

In these, A is an air pump of any convenient kind for supplying air under pressure to the hollow casing B surrounding the 40 cooling chamber N. C indicates any convenient kind of heating device or furnace, K an aspirating chamber, D the chimney from the same, through which the waste gases from the furnace C escape, and C' a 45 pipe or manifold for the passage of air from the jacket B and over the heating device C to the aspirating device in chamber K. E is a tank placed high in any convenient position with a heating device E' underneath. It can however receive its entire 50 heat from the effluent gases of the chimney if desired. In this tank the lead is fused. Any well-known device for delivering lead under pressure can be used, instead of this 55 tank placed on a high level, but I prefer this latter. In any case the lead must be

heated sufficiently to be very fluid, and be kept fluid until it is aspirated as hereafter described. It is well to have a thick layer of carbon to shield the lead from air currents and to prevent oxidation. In order to keep the lead hot in transit, I pass the lead down to aspirator K, hereafter described, by an iron or steel pipe F in the chimney, such pipe being exposed to the heat of the effluent 60 gases. In the tank is a valve Z having a handle Z' whereby the flow of lead down this pipe may be controlled and shut off at any time. It will be noted that the pipe being in the chimney, the temperature of the 65 lead will be increased instead of decreased during its descent. G is a pipe coming from the pump A to the hollow casing B, surrounding chamber N hereafter described and carrying cooling air to the casing where 70 it is heated in turn and from which it is brought by pipe C' to the injector. The injector is shown in Fig. 3 on an enlarged scale, and is made of cast iron or steel in 75 four pieces V, W, X and Y. These are carefully planed at their junctions, and at their orifices and have preferably chipping strips at their junctions so that as the orifices wear, they can be taken down and planed away 80 so as to again reduce the central orifices to 85 a series of fine passages of their original size. H is a long row of small and preferably round orifices evenly spaced for the escape of the liquid lead. I is a very much wider slit at right angles, or nearly so, 90 bringing a blast of heated air from the pipe C'. These two orifices or sets of orifices are 95 parallel and open out into the air as close together as possible, and at right angles to the resultant line of these two jets is a second orifice J for producing a jet of hot air, also brought from the pipe C', said orifice J being placed as near as possible to the two other orifices H and I. A good set of dimensions is 3/8 of an inch for the air slits 100 and a row of holes about 1/50 of an inch wide and 1/10 of an inch apart for the lead, the exact dimensions however should vary with the respective pressures of the lead and air. K is an aspirating and conversion 105 chamber into which these jets discharge, said chamber having a door K' for examining the interior, a scraping hole door K<sup>2</sup> at the bottom, and a sight hole K<sup>3</sup> supplied with a mica window if desired. K<sup>5</sup> is a 110 scraper plate firmly fixed on two shafts K<sup>6</sup> passing through the conversion chamber K

and having two knobs K<sup>7</sup> one at each end, see Fig. 4, so that if any collection of oxid takes place around the injector it can be cut off by forcing the plate from one side of the converter chamber to the other by pulling or hammering on the knobs. L is a further hot air pipe entering the chamber below the injecting device, and having a damper L' worked from the outside, so that the amount of air entering the chamber can be regulated. If unoxidized lead falls into the chamber K the pressure of air must be increased or this opening L more widely opened. M is a pipe leading from chamber K and delivering mixed gases and dust hereafter described to the cooling and settling chamber N. It will be noticed that this pipe passes for six to ten feet up the chimney, then passing a bend on which there is an inspection and cleaning lid M', it descends again at M<sup>2</sup> to chamber N. Settling chamber N has a small exit chamber O supplied with a filter, for filtering out any dust from the escaping gases in a well-known manner yet allowing the filtered gases to escape. The pipe M passes up the chimney so as to continue the heat for a very considerable distance preferably about six to ten feet. P is a conveyer in chamber N slowly or occasionally or continuously put in motion and serving to force the gases to take a circuitous course and prevent a direct draft from pipe M to the exit chamber O; it also draws the deposited dust to the various valves R<sup>2</sup>, hereafter described, as required. The settling chamber N is surrounded by the hollow casing B as shown in Fig. 1. Said casing or air jacket is supplied with a continuous blast of cold air from pump A, and the air preferably is made to take a circuitous course in the jacket or casing by a spiral baffle N'. Jacket B could be dispensed with and larger heating apparatus used at C, but it is useful as saving much useless loss of heat. Q are horizontal carbonating cylinders each of them having a stirring device consisting of a shaft R formed with Archimedean or other blades R' for stirring up the materials. Horizontally disposed and fixed blades R<sup>2</sup> are placed between the blades R' at intervals, said blades R<sup>2</sup> being attached at their ends to the cylinder and having bearings through which shaft R passes. R<sup>4</sup> are valves with measuring devices of any known applicable form for regulating the delivery of the material from the settling chamber N to the series of carbonating cylinders Q. R<sup>3</sup> is a small chamber connected with each carbonating chamber and adapted to contain acetic acid at the bottom. Carbonic acid is passed into the main carbonating cylinders by the pipes R<sup>5</sup> or R<sup>6</sup>. The carbonic acid can thus be passed to cylinders Q directly from the outside if desired through pipe R<sup>8</sup>,

or by pipe R<sup>5</sup> through chamber R<sup>3</sup>. A small heating device R<sup>7</sup> can be placed below this chamber to heat the acetic acid, but this is not as a rule necessary. T is a manhole at the end of each chamber Q out of which the material can fall when finished and T' a similar manhole in chamber N. G' Fig. 3 is one or more steam jets which assist materially in forcing the air through the apparatus and apparently in hydrating the effluent oxid dust. Indeed with steam injectors of air it may be possible to do without a pump altogether, but a pump is desirable as too much steam cools the air.

The mode of operation of this apparatus is as follows:—

The fire C being lighted air is passed through pipe C' either by pump A or steam jet G' or both. As soon as the injector is at about 400° centigrade and the lead is well melted in tank E, the lead is allowed to flow down pipe F and the full blast of air put on.

The hot air passes into the two outside slits at the highest pressure that can be conveniently obtained with this apparatus and the lead passes through the central jets H. A comparatively low pressure, for instance a few ounces to one lb. per square inch on the air can be made to do, but the greater the pressure, the better the apparatus works and the narrower can be the air slits. There can also be further lateral air jets if desired. In the meantime the damper L is slightly opened to admit a further air supply. The operator can determine when the air supply is right by taking out a little of the dust which falls to the bottom of the chamber K and ascertaining whether there is any metallic lead in it. If there be metallic lead, an additional amount of air should be admitted. The lead and air together with some steam from the jets G' passing through the three jets, meet each other with great force at approximately right angles, and the slits being very long and narrow, the lead is divided into an extremely fine even spray, while at the same time the air and steam meeting it cause it to burst into vivid combustion, and to become completely converted into an oxid or more or less hydrated oxid of lead. The air and gases escape through the filtering device at the exit chamber O. The lead compound is deposited in the settling chamber N, and this being surrounded by the cooling jacket B, the lead is soon cooled to from 90° to 140° Fahr. It is desirable to keep the lead hydrated oxid at about 90 to 140 degrees, so that it shall fall into the carbonators Q at this temperature. From the end of the settling chamber conveyer P carries the cooled oxid to any one of the carbonating cylinders Q which happens to be empty or insufficiently filled, the material passing through

one of the valves  $R^4$  for this purpose. In these carbonating cylinders the shafts  $R$  and stirrers  $R'$  are kept in continuous motion. These stirrers and the lining of the entire 5 mixer are preferably made of hard wood well soaked in hot paraffin wax. When the oxid or hydrated oxid has been filled into a chamber  $Q$  to one-fourth or one-fifth of the diameter of the carbonator, and the 10 bottom of the chamber  $R^3$  has been filled to a few inches in depth through a stoppered opening  $R^9$  above with dilute acetic acid and water, carbonic acid is also passed in. At first after the chamber  $Q$  has had the air 15 driven out by the  $CO^2$  it is well to use tolerably strong acetic acid and heat the bottom of chamber  $R^3$  for a time nearly to ebullition so that there shall be plenty of acetic acid in the carbonator  $Q$ , but care should always 20 be taken that the material in the carbonator should never be allowed to get wet to the touch, hence after a time the heat in the little chamber  $R^3$  is brought to about  $100^{\circ}$  Fahr. or under, the degree of heat being 25 regulated so as to always have some atmosphere of acetic acid and of water in the chamber. Practically, from 1 to 2% of acetic acid is desirable per weight of lead operated on. Toward the close, however, of 30 the operation, less acetic acid is used, and the little chamber  $R^3$  is kept colder than near the beginning. From time to time a little of the material is withdrawn from the mixer, and tested. As soon as it is found that it 35 has reached the state of normal white lead, the supply of carbonic acid is stopped, the man-hole door opened, and the blades, which are somewhat archimedean, are allowed to empty the entire chamber, or if desirable the 40 motion of the stirrer is stopped, and the blades being brought to the horizontal the charge is drawn out by scrapers resembling Dutch hoes. If impure carbonic acid be used, which is generally the case, there is an 45 opening  $Q^2$  at the lead dust supply end of each chamber  $Q$  for the escape of waste gases.

In thus describing my invention, I do not bind myself to horizontal carbonators, as vertical or oblique ones could be used, but I prefer the horizontal. In place of acetic acid there are other wellknown catalytes for this purpose that could be used, but they are not so advantageous as acetic acid. I would 55 here mention that a device very similar to my injecting device has already been used on a large scale for making extremely fine pulverulent lead and fine hair of lead, neutral gases, such as a steam blast or nitrogen being used instead of air. Further, that the hydrated oxid of lead formed by my process collected in chamber  $N$  can be used in place of litharge for nearly all purposes for which litharge or pure oxid is used 60 at the present time. If therefore the sup-

ply of lead hydroxid be too large for the various cylinders  $Q$  to carbonate some of the material can be taken from the conveyer through man-hole  $T'$  and used as litharge instead of being passed to chambers  $Q$ . 70

I declare that what I claim is:

1. The process of making white lead, which consists in heating the lead to a degree considerably above its melting point; aspirating it through fine passages of uniform size with highly-heated air, the lead and air being brought into contact under a considerable pressure and the air being sufficient to fully oxidize the lead to monoxid; cooling the oxidized dust thus formed; 75 treating it at from  $90^{\circ}$  to  $140^{\circ}$  F. with carbonic acid and the fumes of acetic acid having sufficient vapor of water to cause the compound to be converted into hydrated white lead; and at the same time agitating 80 the dust.

2. The process of making pure sublimed non-fused lead oxid applicable for making white lead by the dry process, which consists in producing an exceedingly fine spray 90 of globules of uniform size of melted lead; bringing a strong blast of hot air against the effluent lead spray at approximately right angles thereto; and supplying further hot air until the lead is completely oxidized 95 to the state of monoxid.

3. The process of making pure lead monoxid suitable for making white lead by the dry process, which consists in forming melted lead into a fine spray of liquid globules 100 of practically uniform size; aspirating the spray with blasts of heated air, the air being of sufficient quantity to completely oxidize into monoxid the lead spray; continuing the thus formed dust and gases in 105 contact with each other at a high temperature until the lead dust is fully converted into monoxid; and lowering the temperature of the compound thus formed by a cooling air current. 110

4. The process of making pure lead monoxid applicable for making white lead by the dry process, which consists in heating the lead at a head considerably above the place where it is afterward to be oxidized; bringing the lead down through a conduit surrounded by heated gases; passing the lead through fine orifices of equal size; exposing it at the same time to strong blasts of heated air in sufficient quantity to convert 115 the whole of the lead into monoxid; and keeping the resultant gases and dust together at a high heat until all the lead is thoroughly converted into monoxid. 120

5. The process of making white lead, 125 which consists in forming metallic lead into a spray of minute liquid globules of substantially uniform size; aspirating these globules with a quantity of hot air sufficient to thoroughly convert the lead into monoxid; 130

keeping the resultant lead dust and current of gases together until the lead is completely monoxidized; thereafter cooling the dust, with agitation; passing the material 5 still in the the form of dust into a converting chamber having an agitating device; and treating it with carbonic acid and the vapor of a solution of acetic acid while in the dust form and agitated, until it is converted into 10 white lead, whereby every particle is exposed equally to the gaseous reagents.

6. The improvement in the process of making white lead, which consists in taking pure non-fused monoxid of lead in dust 15 form, and without it being allowed to cake; passing it with agitation into an atmosphere containing carbonic acid and the fumes of acetic acid; and agitating it and thus equally exposing every particle to the action of the 20 reagents until it has arrived at the stage of white lead.

7. The process of manufacturing white lead, which consists in exposing pure non-fused monoxid of lead free from metallic

lead in fine dust form, with agitation, to 25 an atmosphere containing carbonic acid and the damp fumes of acetic acid at from 90° to 140° F.; and keeping up the agitation so that every particle shall be uniformly exposed to the reagents until converted into 30 white lead.

8. The improvement in the process of making white lead, which consists in taking pure, non-fused monoxid of lead, free from metallic lead, and in the dust form; and 35 treating it, with agitation, to an atmosphere of carbonic acid and fumes from an aqueous solution of acetic acid, the whole being kept at from about 90° to about 140° F. until it is formed into white lead. 40

In witness whereof, I have hereunto signed my name this 26 day of January, 1915, in the presence of two subscribing witnesses.

WM. P. THOMPSON.

Witnesses:

J. DUCKERS,  
J. McCormick.